

**1**

2,861,958

**PROCESS OF PREPARING A SILICA-ALUMINA-PLATINUM CATALYST**

Wayne Thomas Barrett, Arnold, Md., assignor to W. R. Grace & Co., Norwalk, Conn., a corporation of Connecticut

No Drawing. Application March 30, 1954  
Serial No. 419,931

5 Claims. (Cl. 252—455)

This invention relates to supported platinum catalysts. In one specific aspect, it relates to gasoline reforming catalysts. In another specific aspect, it relates to gasoline reforming processes employing these catalysts. In still another specific aspect, it relates to methods of preparing reforming catalysts.

In the production of motor fuels, it has been found that certain classes of hydrocarbons have higher octane ratings than others. Accordingly, the overall octane rating of a motor fuel would be increased by any treatment which increases the content of these high-octane constituents. By way of illustration, gasoline is made up of hydrocarbons having about 4 to 11 carbon atoms and classified broadly as aromatic, naphthenic, olefinic, paraffinic, and isoparaffinic. The octane numbers of the pure hydrocarbons are a function of their molecular size and chemical nature. In general, it is understood that isoparaffins and aromatics have high octane ratings, naphthenes and mono-olefins intermediate ratings and normal paraffins low ratings. Di-olefins, because of their instability, cannot be tolerated. Thus, in order to produce a gasoline having high anti-knock qualities, it is desirable to have the highest possible content of aromatics and isoparaffins.

Unfortunately, the hydrocarbon cracking reactions by which petroleum distillates are formed do not permit close control over the aromatic content of the distillates so produced. The cracked products can be upgraded (octane-wise) by distillation, but the yield is lowered by the amount of low-octane constituents removed. It is known that straight run naphthas and cracked distillates can be upgraded by catalytic treatments which convert the low-octane compounds to high-octane compounds. This process of upgrading gasolines is referred to as catalytic reforming. The reforming reactions, generally, are dehydrogenation, dehydrocyclization, and isomerization. By these reactions straight chain hydrocarbons are converted to branched hydrocarbons, certain naphthenic constituents are converted to cyclohexanes from which aromatics are formed by dehydrogenation. The entire field of catalytic reforming is rather complex and difficult to interpret but the results are significant.

Efficient reforming of motor fuels requires that there occur a small amount of cracking in order that any heavier-than-gasoline components (distilling above about 400° F.) be cracked to yield lower boiling constituents, which may be subsequently upgraded. It is desirable that reforming reactions be effected with a minimum of

**2**

gas formation and coke deposition since the former reduces the yield and the latter may impair the efficiency of the catalyst. Reforming processes are normally carried out in the presence of hydrogen in order to maintain the gas formation and coke deposition at a minimum. Since hydrogen is formed by the reforming reactions, it is not usually necessary to add extraneous hydrogen to the system except at the start-up.

The prior art has disclosed a number of catalysts as being suitable for reforming gasoline fractions. Among these are platinum or palladium supported on a base which exhibits cracking activity, examples of which are silica-alumina, silica-alumina-zirconia, or silica-magnesia. In the case of silica-alumina bases, the prior art teaches that the alumina content must be 5% or greater in order for the base to have the requisite cracking activity. One type of commercial reforming catalyst is prepared by impregnating a composite silica-alumina base (12%—15% alumina) with a platinum compound, which is subsequently reduced to metallic platinum. In view of the relatively high cost of producing a composite silica-alumina cracking component base, it is desirable to find a catalyst which does not require the use of this type of base. This unfavorable cost factor is made worse by the fact that impregnation techniques are complicated and success is not always assured.

Another type of reforming catalyst is prepared by impregnating an alumina base with a platinum compound, which is subsequently converted to metallic platinum.

Silica gel alone has no cracking activity and has never been used as a base for reforming catalysts. This is unfortunate since granular silica gel is simple to make, while alumina and the composite bases require more extensive procedures. Silica gel is a comparatively low-cost base and a reforming catalyst prepared therefrom would be much cheaper than conventional catalysts.

In accordance with the present invention, it is now possible to prepare an efficient reforming catalyst on a silica gel base.

It is therefore an object of this invention to provide a superior petroleum reforming catalyst. It is another object to provide a method for preparing a reforming catalyst on a silica gel base. It is still another object to provide a process for reforming petroleum fractions. Other objects and advantages of the present invention will be apparent to those skilled in the art from the following detailed description and the appended claims.

The novel catalyst of the present invention comprises a silica gel base supporting the requisite amount of platinum and a very small amount of alumina deposited on the silica gel simultaneously with the platinum. The catalyst is prepared by impregnating silica gel with an aqueous solution containing aluminum and chloroplatinate ions, drying the impregnated silica gel, and converting the aluminum and platinum constituents to metallic platinum and alumina.

It has been discovered that silica gel impregnated with about 0.05—5 wt. percent of platinum and about 0.01—1.0 wt. percent alumina from aqueous solutions of aluminum chloroplatinate, postulated as  $Al_2(PtCl_6)_3$ , or mixed aqueous solutions of an aluminum salt and chloroplatinic acid

yields, upon reduction, a catalyst which has the desired reforming characteristics of the conventional platinum on silica-alumina or platinum on alumina catalysts and which is considerably cheaper than such catalysts.

Because of its high cost, the amount of platinum in any catalyst will always be the minimum amount that will give the desired results. The platinum content will normally be held to about 0.2-1.0 weight percent and the alumina content to about 0.1-0.5 weight percent since efficient reforming can be accomplished at these concentrations.

The silica gel useful in the present invention is a prepared form of amorphous silicon dioxide having an extremely porous structure. It is extensively described in the scientific literature and is described in the patent literature as early as U. S. Patent No. 1,297,724 of Walter A. Patrick. It may be prepared by mixing predetermined amounts of a mineral acid, e. g. sulfuric acid, and a soluble silicate, e. g. sodium silicate, allowing the resulting mixture to set to a jelly-like hydrogel, washing the hydrogel to remove soluble salts and drying the washed material. The dried material may be crushed and screened to the desired particle size. It is usually given an activation treatment, which comprises heating the dried material to a temperature slightly in excess of the temperature at which the finished material is to be used. Silica gel is a well-known article of commerce and is widely used as a desiccant, a carrier for other catalytic agents and as a filler in paints and varnishes. The material prepared in the described manner is in the form of hard, rugged, irregularly shaped granules. These may be used as the base for preparing the catalyst of the present invention or they may be formed into shapes as desired. Dried silica gel is an excellent adsorbent and can be readily impregnated with aqueous solutions.

Platinum on silica gel catalysts have been prepared heretofore by impregnating silica gel with chloroplatinic acid. These catalysts are used for sulfur dioxide oxidation. However, they have no value as hydrocarbon reforming catalysts and are not to be confused with the catalysts of the present invention which also contain very small amounts of alumina and are prepared by different methods.

In one embodiment of the present invention the silica gel base is impregnated with aluminum chloroplatinate. This compound is the aluminum salt of chloroplatinic acid and may be formed by obvious chemical reactions. A convenient method is to add a relatively pure hydrous alumina in excess to an aqueous solution of chloroplatinic acid. The solution dissolves alumina to give a yellow solution containing the undissolved excess of alumina, which is removed by filtration to give a clear solution of aluminum chloroplatinate. The silica gel base is then impregnated with the aluminum chloroplatinate solution, using any convenient impregnation technique. The concentration of aluminum chloroplatinate in the impregnating solution is adjusted to give the desired platinum content to the finished catalyst when the silica gel has been saturated to the extent obtained by the specific procedure.

If the empirical formula for aluminum chloroplatinate is  $\text{Al}_2(\text{PtCl}_6)_3$ , this formula dictates that the alumina content of a catalyst prepared by the above method be approximately one-fifth the platinum content. Thus, if the platinum content is 0.5 weight percent, the alumina content is about 0.1 weight percent. In practice, the alumina content from aluminum chloroplatinate prepared by the above procedure is somewhat higher, as much as three or four times the stoichiometric. This slight excess of alumina is not of any consequence and does not appear to have any detrimental effect on the catalyst. However, as will be indicated later, reducing the alumina content below the stoichiometric quantity has a decidedly adverse effect. Thus, pure aluminum

chloroplatinate may be used as the impregnant or the more easily prepared but somewhat less pure material prepared as indicated above may be used.

In addition to aluminum chloroplatinate, other solutions containing aluminum and chloroplatinate ions may be employed to impregnate the silica gel with alumina and platinum simultaneously. Mixed solutions of an aluminum salt and chloroplatinic acid are entirely satisfactory.

10 In a specific embodiment of the present invention the impregnant comprises a mixed solution of aluminum chloride and chloroplatinic acid. This mixed solution permits greater flexibility of control over the alumina content or the ratio of platinum to alumina in the final catalyst, by varying the quantity of aluminum chloride in the mixed solution. In some instances, this method may be preferred to other methods.

The aluminum and chloroplatinate ion containing impregnating solutions may be applied to the silica gel base 20 by spraying a given quantity of base with sufficient solution to give the desired platinum and alumina content to the finished catalyst. When the spray technique is used, the concentration of the aluminum and chloroplatinate ions in the solution should be such that the gel is brought to the stage of incipient wetness. This insures uniform dispersion of the platinum throughout the base. The impregnated base is dried and the aluminum and chloroplatinate constituents are converted to alumina and platinum by known methods.

30 As an alternative to the spray technique, the silica gel base may be immersed in the impregnating solution until it becomes saturated, following which, it is drained to remove excess liquid and dried and reduced. In using this method, it is necessary to take into consideration the 35 unexplained phenomenon that silica gel appears to repel the chloroplatinate ions so that there is a selective adsorption of water from these impregnating solutions, resulting in an increase in concentration of chloroplatinate ions during contact with the silica gel. Due allowance 40 for this phenomenon can be made by carrying out a trial impregnation. Because of this phenomenon, the silica gel base is allowed to remain in contact with the impregnant for only sufficient time to adsorb the necessary amount of impregnant.

45 A convenient method of drying the impregnated silica gel is to tumble it in a stream of heated air. Another method is to pass a stream of heated air or gas through a bed of the impregnated gel. The dried gel is reduced with hydrogen in a manner to give a silica gel impregnated with the small amounts of platinum and alumina. Alternatively, the hydrogen reduction may be substituted by thermal decomposition or other convenient means of converting the aluminum and chloroplatinate constituents to alumina and metallic platinum.

55 The present invention will be further illustrated by the following non-limiting examples:

#### EXAMPLE 1

60 Three series, designated as Series A, B, and C, of supported platinum catalysts were prepared. Series A and C comprise five catalysts containing approximately 0.05, 0.10, 0.20, 0.40 and 0.80 weight percent platinum. Series B comprises three catalysts containing approximately 0.15, 0.30, and 0.60 weight percent platinum. The catalysts of each series were prepared by the same general methods as indicated hereafter:

70 Series A—Chloroplatinic acid on silica-alumina granules  
Series B—Chloroplatinic acid on silica gel  
Series C—Aluminum chloroplatinate on silica gel

75 The silica-alumina base contained approximately 15.5 percent alumina and was prepared by impregnating

washed silica hydrogen with aluminum nitrate and drying and calcining the resulting material and then steam deactivating the calcined material to a 16.5 weight percent cracking activity. The finished base had a surface area of 51 m.<sup>2</sup>/g. and was similar to the bases used in commercial catalysts.

#### Series A

The catalysts of Series A were prepared by soaking the silica-alumina base in a solution of chloroplatinic acid of suitable concentration for eight days at approximately 180° F., using a closed container to prevent evaporation of liquid. The concentrations of the platinum solutions were selected to give the desired platinum content in the finished catalyst, as determined by the adsorption characteristics of this base. At the end of the impregnation period, the jars were cooled, the excess liquid was drained off and the impregnated granules were washed three times with distilled water to remove soluble platinum. Following this, the granules were dried in an oven for 48 hours at 230° F. and then heated to about 450° F. for about 1½ hours in a stream of dry oxygen-free nitrogen. The dried material was reduced for two hours at 450° F. in a stream of dry, oxygen-free hydrogen. The reduced catalysts were finally cooled to ambient temperatures in a hydrogen stream.

#### Series B

The catalysts of Series B were prepared by impregnating a commercial grade of silica gel identified as The Davison Chemical Corporation's Grade 40 silica gel. The properties of this material are indicated hereafter:

SiO<sub>2</sub> (dry basis) 99.60% min.  
Water soluble 0.50% max.  
Density 40-45 lbs. per cu. ft.

An 8-12 mesh fraction of this silica gel was heated for four hours at 1200° F. following which it was cooled and sprayed with the predetermined amount of chloroplatinic acid solution to give the desired platinum content in the finished catalyst. The thus impregnated material was dried and reduced in the manner described for Series A.

#### Series C

The catalysts of Series C were prepared by the same method of impregnation of the same silica gel base described for those of the Series B, but using the aluminum chloroplatinate impregnating solution of this invention. This solution was prepared by dissolving freshly precipitated hydrous alumina in a solution of chloroplatinic acid. Drying and reduction of the catalysts were carried out in the same manner employed for the catalysts of Series A and B.

The catalysts of the foregoing series were prepared under very carefully controlled conditions to insure that, apart from fundamental differences, the procedures followed were as nearly identical as possible. All of the catalysts were analyzed for total platinum to facilitate comparison between the catalysts at the same platinum level.

The activities of the catalysts in each series were examined by the methylcyclopentane (hereinafter designated as MCP) method. In carrying out this test, a mixture of MCP and hydrogen was passed over 50 ml. of 8-12 mesh catalyst in a tubular reactor at a temperature of 860° F. and a pressure of 500 lbs./sq. in. The hydrogen to hydrocarbon ratio was 6 to 1, and the liquid hourly space velocity was 2.25. Isomerization-dehydrogenation reactions result in the conversion of MCP to benzene. The activity of each catalyst was measured by the yield

of benzene obtained during the second hour of the test. Gases from the reactor were passed through a water trap at 32° F. and thence through a Dry Ice trap. The benzene content of the liquid product was determined by examination with a Beckman spectrophotometer. Losses comprised uncondensable gases. The results of these tests appear in the following table.

TABLE I

| Catalyst No. | Weight percent Platinum | Weight percent Yield by MCP Test |         |
|--------------|-------------------------|----------------------------------|---------|
|              |                         | Liquid Product                   | Benzene |
| 15           |                         |                                  |         |
| Series A:    |                         |                                  |         |
| 1            | 0.045                   | 84.7                             | 11.4    |
| 2            | .105                    | 84.0                             | 14.3    |
| 3            | .183                    | 95.4                             | 16.1    |
| 4            | .366                    | 93.7                             | 14.1    |
| 20           | .624                    | 89.8                             | 14.5    |
| Series B:    |                         |                                  |         |
| 1            | 0.155                   | 81.7                             | 3.4     |
| 2            | .316                    | 91.4                             | 4.4     |
| 3            | .636                    | 80.1                             | 4.6     |
| 25           |                         |                                  |         |
| Series C:    |                         |                                  |         |
| 1            | 0.044                   | 79.3                             | 2.4     |
| 2            | .125                    | 92.2                             | 5.1     |
| 3            | .178                    | 91.5                             | 7.7     |
| 4            | .355                    | 95.8                             | 10.7    |
| 5            | .688                    | 91.9                             | 11.9    |

The MCP activities of Series C catalysts, prepared by the method of this invention, increased with increased platinum content, the yield of benzene reaching a value of 11.9% at about 0.7% platinum. These activities were somewhat lower than those of Series A catalysts (extended chloroplatinic acid impregnation of a silica-alumina base at 180° F.). However, the yields of liquid product attained with Series C catalysts were superior in most instances to those with Series A catalysts.

Series B catalysts (chloroplatinic acid-silica gel) all showed very low activities in striking contrast to the activities of the catalysts prepared according to the present invention, which contain only a few hundredths of a percent more alumina.

#### EXAMPLE 2

In order to compare the reforming ability of the catalysts of Example 1 under actual reforming conditions, 200 hour tests were carried out on three Series A, one Series B, and three Series C catalysts. These tests comprised passing a mixture of hydrogen and an East Texas Naphtha having the following properties:

|     | ASTM distillation:             | ° F. |
|-----|--------------------------------|------|
| 55  | Overpoint                      | 178  |
| 10% |                                | 212  |
| 50% |                                | 255  |
| 90% |                                | 319  |
| 95% |                                | 330  |
| 60  | Endpoint                       | 350  |
|     | API Gravity @ 60° F.: 56-57.   |      |
|     | CFR-Research Octane No. 54-57. |      |

in a tubular reactor over a bed of 75 ml. of 8-12 mesh catalyst, which had been activated at 900° F. for one hour. The inlet temperature was 930° F. and the pressure 500 lbs./sq. in. The hydrogen to hydrocarbon ratio was 12.6 to 1 and the liquid hourly space velocity 3.0.

The activity and stability of each catalyst was assessed by considering the Research Octane numbers of the reformates produced after 72 and 200 hours. A catalyst is regarded as good if, under the above conditions, the octane number of the reformate after 72 hours is 88 or greater, and the decrease in octane number between 72

and 200 hours does not exceed about 2.5 units. The following table illustrates the results of these tests:

TABLE 2

| Catalyst         | Weight Percent Platinum | CFR-RO No. at 4 lb. R. V. P. |         |          | Volume Percent Yield at 88.0 CFR-RO | API Gravity @ 60° F. |         |  |
|------------------|-------------------------|------------------------------|---------|----------|-------------------------------------|----------------------|---------|--|
|                  |                         |                              |         |          |                                     | 72 hr.               | 200 hr. |  |
|                  |                         | 72 hr.                       | 200 hr. | Decrease |                                     | 72 hr.               | 200 hr. |  |
| <b>Series A:</b> |                         |                              |         |          |                                     |                      |         |  |
| No. 3            | 0.183                   | 88.0                         | 84.0    | 4.0      | 86                                  | 51.4                 | 51.8    |  |
| No. 4            | .366                    | 87.8                         | 86.5    | 1.3      | 85                                  | 50.2                 | 50.4    |  |
| No. 5            | .624                    | 89.0                         | 86.8    | 2.2      | 85                                  | 50.8                 | 50.9    |  |
| <b>Series B:</b> |                         |                              |         |          |                                     |                      |         |  |
| No. 3            | .636                    | 78.3                         | 77.1    | 1.2      | 86                                  | 52.6                 | 52.1    |  |
| <b>Series C:</b> |                         |                              |         |          |                                     |                      |         |  |
| No. 3            | .178                    | 82.5                         | 81.1    | 1.4      | 86                                  | 52.0                 | 51.5    |  |
| No. 4            | .355                    | 88.0                         | 86.0    | 2.0      | 86                                  | 51.4                 | 51.2    |  |
| No. 5            | .688                    | 88.8                         | 87.4    | 1.4      | 84                                  | 53.2                 | 52.2    |  |

Only four of the seven catalysts tested met the 88.0 octane requirement at 72 hours, and/or a decrease of less than 2.5 units after 200 hours. These were Numbers 4 and 5 of Series A, chloroplatinic acid-silica-alumina base, and Numbers 4 and 5 of Series C prepared by the present invention. Although Series C Catalyst No. 3 did not produce an 88 octane reformate, the increase in octane rating of the feed from 56-57 to 81-82 is indicative of its substantial reforming ability. To determine the yield-octane

described in Example 2. A mixture of hydrogen and the East Texas Naphtha of Example 2 was passed in a tubu-

lar reactor over 75 ml. of 8-12 mesh catalyst which had been activated for two hours at 1000° F. The inlet temperature was 940° F., and the pressure 500 lbs./sq. in. The liquid hourly space velocity was 3.0 and the hydrogen to hydrocarbon ratio 10.0 to 1. CFR Research Octane Numbers and API Gravities of the reformates were measured after 72 and 200 hours on stream. Volume percent yield was determined at CFR-RO No. 89.5. The following table presents the results of these tests.

TABLE 3

| Catalyst                                               | Weight Percent |                                | CFR-RO No. |         | Volume Percent Yield at 89.5 octane | API Gravity @ 60° F. |         |
|--------------------------------------------------------|----------------|--------------------------------|------------|---------|-------------------------------------|----------------------|---------|
|                                                        | Pt             | Al <sub>2</sub> O <sub>3</sub> | 72 hr.     | 200 hr. |                                     | 72 hr.               | 200 hr. |
| D: Al <sub>2</sub> (PtCl <sub>6</sub> ) <sub>3</sub>   | 0.36           | 0.26                           | 88.7       | 86.9    | 86.8                                | 51.9                 | 51.9    |
| E: H <sub>2</sub> PtCl <sub>6</sub> /AlCl <sub>3</sub> | 0.43           | 0.20                           | 90.6       | 87.9    | 88                                  | 52.4                 | 52.2    |

relationship in cases where an octane of 88 was closely approximated but not attained, the yield which would be expected at 88 was estimated by applying a correction factor.

Table 2 indicates that the octane number of the reformate after 200 hours increases as the platinum content of Series A and Series C catalyst is increased. The table further shows that Series A and Series C catalysts containing approximately the same weight percent platinum produce reformates after 200 hours of approximately the same octane rating. The optimum platinum content of both catalysts appears to be about 0.4-0.5 weight percent. It is also evident from Table 2 that the yield from Series C catalysts, which contain less than 1 weight percent alumina on the silica gel support, are as good as the yields attainable with Series A catalysts, the silica-alumina base of which contains 15.5 weight percent alumina.

The API gravity measurements of the reformates prepared with the catalysts of this invention after 72 and 200 hours are fairly constant. This indicates that the novel catalyst is quite stable after 200 hours on stream.

#### EXAMPLE 3

In order to illustrate two methods of preparing the catalyst of this invention, two silica gel base catalysts, designated as D and E, were prepared and tested under actual reforming conditions. Catalyst D was prepared in accordance with the method set forth in Example 1 for Series C catalyst. Catalyst E was likewise prepared in accordance with the method of Example 1, Series C, except that the impregnant was a mixed solution of chloroplatinic acid and aluminum chloride. By calculated addition of aluminum chloride to the chloroplatinic acid solution prior to impregnation, the alumina and platinum contents of Catalyst E were made to closely approximate those of Catalyst D.

Reforming test conditions were similar to those de-

40 These data clearly indicate that catalysts prepared either by impregnation of a silica gel base with aluminum chloroplatinate or with a solution containing aluminum chloride and chloroplatinic acid are entirely satisfactory reforming catalysts. They both produce high yields of high octane reformates, and are both highly stable catalysts.

45 In addition to aluminum chloroplatinate and a mixed solution containing aluminum chloride and chloroplatinic acid, other solutions containing aluminum ions and chloroplatinate ions may be employed to impregnate the silica gel according to this invention. As a practical matter, certain aluminum salts other than aluminum chloride may be combined with chloroplatinic acid to form a satisfactory impregnating solution, e. g. aluminum nitrate. The choice of aluminum salts, however, is necessarily restricted to those which do not contain ions which will poison the final catalyst or reduce its initial activity. Acceptable aluminum salts are those whose anions will be removed from the catalyst during

55 hydrogen reduction or calcination as the case may be.

60 The reforming process employing the catalyst prepared in accordance with the present invention will be effected at a temperature of about 600° to about 1000° F., at a pressure of about 50-1000 p. s. i. and at a liquid hourly space velocity of about 0.5-10. The liquid hourly space velocity is defined as the volume of oil per hour per volume of catalyst in the reaction zone. Sufficient hydrogen will usually be produced in the reforming reaction to furnish the hydrogen required in the process, and therefore it is usually unnecessary to introduce extraneous hydrogen except at the start up. In order to assure a sufficient hydrogen atmosphere in the reaction zone after start up, hydrogen produced is usually recycled. The hydrogen present in the reaction zone will be within the range of from about 0.5 to about 15 mols 65 of hydrogen per mol of hydrocarbon. The exact tem-

perature, pressure, space velocity and hydrogen to hydrocarbon ratio used in any given operation will depend upon the particular gasoline fraction being treated and the products desired.

I claim:

1. A method for preparing a silica gel base catalyst suitable for reforming gasoline fractions which comprises impregnating silica gel with an aqueous solution of aluminum chloroplatinate in amount sufficient to incorporate in said gel about 0.05-5.0 weight percent platinum and 0.01-1.0 weight percent alumina, drying the impregnated gel, and converting the adsorbed platinum compound to alumina and metallic platinum.

2. A method for preparing a silica gel base catalyst suitable for reforming gasoline fractions which comprises activating silica gel at a temperature above that at which reforming is carried out, impregnating the activated gel with an aqueous solution of aluminum chloroplatinate in amount sufficient to incorporate in said gel about 0.05-5.0 weight percent platinum and 0.01-1.0 weight percent alumina, drying the impregnated gel, and converting the adsorbed platinum compound to alumina and metallic platinum.

3. A method according to claim 2 wherein the catalyst is thermally activated following conversion of the adsorbed constituents.

4. A method for preparing a silica gel base catalyst suitable for reforming gasoline fractions which comprises heating silica gel at a temperature of about 1200° F. for a period of about 4 hours and thereby activating said

5 gel, impregnating the activated gel with an aqueous solution of aluminum chloroplatinate in amount sufficient to incorporate in said gel about 0.05-5.0 weight percent platinum and 0.01-1.0 weight percent alumina, drying the impregnated gel, and converting the adsorbed platinum compound to alumina and metallic platinum.

10 5. A method for preparing a silica gel base catalyst suitable for reforming gasoline fractions which comprises heating silica gel granules having a particle size of about 15 8-12 mesh at a temperature of about 1200° F. for a period of about 4 hours and thereby activating said gel, impregnating the activated gel with an aqueous solution of aluminum chloroplatinate in amount sufficient to incorporate in said gel about 0.05-5.0 weight percent platinum and 0.01-1.0 weight percent alumina, drying the impregnated gel, and reducing the dried gel in an atmosphere of hydrogen.

References Cited in the file of this patent

UNITED STATES PATENTS

|           |                       |               |
|-----------|-----------------------|---------------|
| 2,005,412 | Connolly et al. ----- | June 18, 1935 |
| 2,437,532 | Huffman et al. -----  | Mar. 9, 1948  |
| 2,452,198 | Kennedy et al. -----  | Oct. 26, 1948 |
| 2,470,142 | Chapman et al. -----  | May 17, 1949  |
| 2,550,531 | Ciapetta -----        | Apr. 24, 1951 |
| 2,589,189 | Ciapetta et al. ----- | Mar. 11, 1952 |
| 2,635,123 | Kennedy -----         | Apr. 14, 1953 |
| 2,662,861 | Riblett et al. -----  | Dec. 15, 1953 |
| 2,663,620 | Haensel -----         | Dec. 22, 1953 |